

Patented Oct. 9, 1928.

1,686,540

# UNITED STATES PATENT OFFICE.

CLARENCE B. WHITE, OF MONTCLAIR, NEW JERSEY, ASSIGNOR TO VIVATEX PROCESSES, INC., OF LODI, NEW JERSEY, A CORPORATION OF NEW JERSEY.

## MINERAL DYEING.

No Drawing.

Application filed December 23, 1926. Serial No. 156,766.

In so-called "iron dyeing" of textile materials (including in the latter term not only fabrics of all kinds but also fibres, yarns, threads, etc.) to produce the well known khaki and Hong Kong shades, the practice heretofore has been to impregnate the material with a ferrous compound and at a later stage subject the material to an oxidizing agent for the purpose of converting the ferrous compound into the ferric state. This step, known as aging, is of the highest importance in prior methods, since the fastness of the color depends upon the extent of the oxidation of the ferrous compound, but to carry the oxidation to completion by the method indicated is exceedingly difficult if not impossible, and in any case it is slow and inefficient. Efforts have also been made to dye with a ferric compound. So far as I am aware the attempts have not been successful since the only ferric compounds sufficiently soluble to form a dye bath of adequate concentration are nitrate, chloride and sulfate or their derivations, which are prone to dissociate upon drying, thereby setting free the acid radical with the result that the textile material is damaged or "tendered". The organic ferric salts which produce but little, and in some cases no, tendering effect, namely the acetate, tartrate, etc., are of such slight solubility that they have not heretofore been usable for the production of pronounced or deep shades of color. Ferric formate is soluble in cold water but hydrolyzes in warm or hot water.

I have accordingly been led to devise my present invention, which has for its chief object to provide a dyeing process by which non-tendering ferric salts, mostly organic in nature, can be effectively employed for producing dark as well as light shades of color. To this and other ends the invention comprises the novel features hereinafter described.

The invention is based upon the observation that the solubility of organic salts of iron and other metals, as for example ferric acetate, tartrate, and oxalate, (and in the case of ferric formate its solubility in warm water without hydrolyzing) can be materially increased by formic or equivalent acid, as acetic, tartaric (racemic and other derivatives), and succinic. The solubilizing acid may be added to the dye bath before or

after the ferric salt, but in either case the latter can be dissolved in amount sufficient to produce very deep fast shades without damage or tendering of the cellulose material. From one to five per cent of formic acid, calculated on the total weight of the bath, is in general sufficient to give a degree of solubility adequate for the production of shades of a depth or strength scarcely obtainable by the use of ferrous salts. Alkali salts such as sodium formate, ammonium formate, etc., exert a less degree of solvent stimulation. The solution of difficulty soluble basic salts of aluminum, copper, thorium, zirconium, etc., as for instance their basic acetates, is also stimulated in the same manner, and in the case of the aluminum, thorium and zirconium salts named such stimulation is necessary since they are all insoluble in water, or nearly so.

In carrying out my invention in the preferred way the ferric salt may be dissolved directly in a solution of formic acid or other stimulant, but it is more practical, especially where the salt to be used for the dyeing is ferric acetate, to prepare the dye liquor from a cheap and abundant ferrous salt, such as "copperas" or ferrous sulfate. The latter is oxidized in its solution by an oxidizing agent such as sodium or potassium chlorate, sodium or potassium di-chromate, nitric acid, sodium or potassium permanganate, etc. The alkali metal chlorates are markedly efficient for the purpose but do not appear to be greatly superior to the di-chromates, the only apparent disadvantage of the latter being that they introduce chrome salts into the solution when such salts may not be desirable. The amount of oxidizing agent required depends of course upon the amount of ferrous salt to be oxidized.

When the ferrous sulfate in solution has been oxidized to the ferric state, preferably completely, the formic acid is added to the liquor in amount dependent upon the desired concentration of the dye bath. The object and effect of the formic acid addition is to retain in solution or cause solution of ferric acetate formed in the next step. As stated above, one to five per cent of formic acid is ordinarily sufficient. After this addition the sulfuric acid, free or combined, is removed from the liquor by means of a soluble salt (say acetate, formate, succinate or tartrate), of barium, calcium, lead,

or other element, capable of reacting with the sulfuric acid or sulfate present in the liquor to form an insoluble sulfate. Barium salts are preferred because of the insolubility of barium sulfate, and the most convenient salt for the purpose is barium acetate, but other acetates are sufficiently effective for practical purposes. Using barium acetate, for example, the resulting reaction produces ferric acetate and barium sulfate. The latter is readily separated from the liquor by filtration.

As stated, the presence of the formic acid or other suitable substance, preferably an organic acid, enables the liquor to retain the acetate or other ferric salt in solution, so that the free and combined sulfuric acid can be removed as described, without the ferric salts being carried down with the insoluble barium sulfate or other sulfate, as would happen if a solvent stimulant were not added prior to the sulfate precipitation. It is, however, feasible to effect the precipitation of sulfates first, and then re-dissolve the precipitated ferric salts with the aid of the solubilizing agent, but the course first described is more advantageous.

After the insoluble sulfates are removed, as by filtration, or otherwise, the ferric dye bath can be used in the customary way, the textile material being passed through the bath and then squeezed to eliminate the excess liquor, the impregnated material usually absorbing about seventy per cent of its own weight. The squeezed material is then dried, preferably on drums. Festooning is possible, though not as economical as the other method of drying.

The impregnated and dried material is now passed through a hot alkali solution, say caustic soda or soda ash (sodium carbonate) or both, or soda ash and soap, preferably at about 80 to 100° C., or cold ammonia solution, of sufficient concentration, readily determinable, to decompose without waste ferric salts and accompanying compounds (for example chromium salts) and form an insoluble iron compound or compounds, as hydroxide, carbonate and oleate, in and upon the fibres of the material. The latter is then washed thoroughly and dried.

It will be noted that the slow and inefficient aging process, or oxidation after impregnation, is unnecessary in the above method. The ability to secure a completely oxidized deposit on the cloth or other material makes possible a degree of uniformity of shade that is difficultly if at all obtainable by the prior methods. At the same time the greater degree of oxidation, substantially complete if desired, renders the shade correspondingly faster, especially to rain and atmospheric agencies in general, and to laundering, and also enables a given shade to be produced with less expenditure of

metallic salts, thereby giving marked economy of operation.

It is to be understood that the invention is not limited to the procedure and details herein specifically described but can be carried out in other ways without departure from its spirit.

I claim—

1. In mineral dyeing of textile material, the steps comprising forming with the aid of 75 a solvent stimulant a solution of a difficultly soluble metallic salt, and impregnating the textile material with the solution.

2. In mineral dyeing of textile material, 80 the steps comprising forming with the aid of a solvent stimulant a solution of a difficultly soluble iron salt, impregnating the textile material therewith, and treating the material to remove from the absorbed iron salt the acid radical thereof and convert the 85 salt into another insoluble compound.

3. In mineral dyeing of textile material, 90 the steps comprising forming a solution of a metallic sulfate; removing sulfuric acid from the solution by forming therewith an insoluble sulfate and simultaneously forming with the metal of the first mentioned salt another and difficultly soluble salt of the same, in the presence of a solvent stimulant whereby the difficultly soluble salt is 95 dissolved to form a dye liquor; impregnating the textile material with the dye liquor; and treating the textile material to remove the acid radical from the salt absorbed there- 100 by and form another insoluble compound.

4. In mineral dyeing of textile material, 105 the steps comprising forming with the aid of a solvent stimulant a solution of ferric acetate, and impregnating the textile material therewith.

5. In mineral dyeing of textile material, 110 the steps comprising treating ferric sulfate, in solution and in the presence of a solvent stimulant, with an acetate capable of reacting with the ferric sulfate to form ferric acetate in solution and an insoluble sulfate; and treating the textile material with the ferric acetate solution.

6. In mineral dyeing of textile material, 115 the steps comprising treating ferric sulfate, in solution and in the presence of a solvent stimulant, with an acetate capable of reacting with the ferric sulfate to form ferric acetate in solution and an insoluble sulfate; treating the textile material with the ferric acetate solution, and converting the absorbed ferric acetate into another insoluble iron compound.

7. In mineral dyeing of textile material, 125 the steps comprising forming with the aid of a solvent stimulant a solution of an otherwise difficultly soluble metallic salt of an organic acid, and impregnating the textile material with the solution.

8. In mineral dyeing of textile material, 130

the steps comprising forming with the aid of a solvent stimulant a solution of an otherwise difficultly soluble organic salt of iron, and impregnating the textile material with

5 the solution.

9. In mineral dyeing of textile material, the steps comprising forming with the aid of formic acid as a solvent stimulant a solution of ferric acetate, and impregnating the

10 textile material with the solution.

10. In mineral dyeing of textile material, the steps comprising oxidizing ferrous sulfate in solution to the ferric state, mixing therewith a solvent stimulant and a solution

15 of a suitable acetate to form ferric acetate in solution and an insoluble sulfate, treating the textile material with the ferric acetate solution, and thereafter treating the textile material with an alkali to remove the

20 acetic acid radical from the absorbed ferric salt and form another iron compound.

11. In mineral dyeing of textile material,

the steps comprising forming a ferrous sulfate solution, treating the same with alkali metal chlorate to oxidize the ferrous salt to 25 the ferric state, treating the ferric sulfate solution with a suitable acetate in the presence of formic acid to form ferric acetate in solution and an insoluble sulfate, treating the textile material with the ferric acetate solution, and thereafter treating the textile material with an alkali solution.

12. In mineral dyeing of textile material, the steps comprising oxidizing ferrous sulfate in solution to the ferric state, mixing 35 therewith formic acid and a barium acetate solution to form ferric acetate in solution and barium sulfate, treating the textile with the ferric acetate solution, and thereafter converting the absorbed ferric acetate into 40 another iron compound.

In testimony whereof I hereto affix my signature.

CLARENCE B. WHITE.